



US008749339B2

(12) **United States Patent**  
**Ogawa et al.**

(10) **Patent No.:** **US 8,749,339 B2**  
(45) **Date of Patent:** **\*Jun. 10, 2014**

(54) **COIL-TYPE ELECTRONIC COMPONENT AND PROCESS FOR PRODUCING SAME**

(75) Inventors: **Hideki Ogawa**, Gunma (JP); **Atsushi Tanada**, Gunma (JP); **Hitoshi Matsuura**, Takasaki (JP); **Kiyoshi Tanaka**, Gunma (JP); **Hiroshi Kishi**, Takasaki (JP); **Kenji Kawano**, Takasaki (JP)

(73) Assignee: **Taiyo Yuden Co., Ltd.**, Tokyo (JP)

(\*) Notice: Subject to any disclaimer, the term of this patent is extended or adjusted under 35 U.S.C. 154(b) by 0 days.

This patent is subject to a terminal disclaimer.

(21) Appl. No.: **13/642,467**

(22) PCT Filed: **Apr. 26, 2011**

(86) PCT No.: **PCT/JP2011/060106**

§ 371 (c)(1),  
(2), (4) Date:

**Nov. 16, 2012**

(87) PCT Pub. No.: **WO2011/136198**

PCT Pub. Date: **Nov. 3, 2011**

(65) **Prior Publication Data**

US 2013/0200970 A1 Aug. 8, 2013

(30) **Foreign Application Priority Data**

Apr. 30, 2010 (JP) ..... 2010-105552  
Apr. 18, 2011 (JP) ..... 2011-091879

(51) **Int. Cl.**

**H01F 27/28** (2006.01)  
**H01F 27/02** (2006.01)  
**B05D 5/12** (2006.01)

(52) **U.S. Cl.**

USPC ..... **336/233; 336/83; 427/116**

(58) **Field of Classification Search**

USPC ..... 336/83, 233, 234; 427/116; 252/62.51, 252/62.54; 428/328, 329, 323, 492; 419/5; 148/105, 304

See application file for complete search history.

(56) **References Cited**

U.S. PATENT DOCUMENTS

4,129,444 A 12/1978 Dreyer et al.  
5,522,946 A 6/1996 Tomita et al.

(Continued)

FOREIGN PATENT DOCUMENTS

CN 101308719 A 11/2008  
CN 101927344 A 12/2010

(Continued)

OTHER PUBLICATIONS

Non-Final Rejection issued by U.S. Patent and Trademark Office, dated Aug. 6, 2013, related U.S. Appl. No. 13/348,926.

(Continued)

*Primary Examiner* — Alexander Talpalatski

*Assistant Examiner* — Mangtin Lian

(74) *Attorney, Agent, or Firm* — Law Office of Katsuhiro Arai

(57) **ABSTRACT**

A coil-type electronic component has a coil inside or on the surface of its base material wherein the base material in the coil-type electronic component is constituted by a group of grains of a soft magnetic alloy containing iron, silicon and other element that oxidizes more easily than iron; the surface of each soft magnetic alloy grain has an oxide layer formed on its surface as a result of oxidization of the grain; this oxide layer contains the other element that oxidizes more easily than iron by a quantity larger than that in the soft magnetic alloy grain; and grains are bonded with one another via this oxide layer. The coil-type electronic component can be produced at low cost and combines high magnetic permeability with high saturation magnetic flux density.

**17 Claims, 6 Drawing Sheets**



|                              |                         |                   |    |                |          |
|------------------------------|-------------------------|-------------------|----|----------------|----------|
| (56)                         | <b>References Cited</b> |                   |    |                |          |
| <b>U.S. PATENT DOCUMENTS</b> |                         |                   |    |                |          |
| 6,392,525 B1                 | 5/2002                  | Kato et al.       | JP | 2001-011563 A1 | 1/2001   |
| 6,764,643 B2                 | 7/2004                  | Sagawa et al.     | JP | 2001-118725 A1 | 4/2001   |
| 6,784,782 B2                 | 8/2004                  | Inoue et al.      | JP | 2002-305108 A1 | 10/2002  |
| 6,814,928 B2                 | 11/2004                 | Sagawa et al.     | JP | 2002-313620 A1 | 10/2002  |
| 7,422,697 B2                 | 9/2008                  | Takahashi et al.  | JP | 2002-343618 A1 | 11/2002  |
| 7,446,638 B2                 | 11/2008                 | Nogi              | JP | 2007-019134 A1 | 1/2007   |
| 8,018,313 B2                 | 9/2011                  | Tada et al.       | JP | 2007-027354 A  | 2/2007   |
| 8,416,051 B2                 | 4/2013                  | Matsuura et al.   | JP | 2007-027354 A1 | 2/2007   |
| 2004/0140016 A1              | 7/2004                  | Sakamoto et al.   | JP | 2007-123703 A1 | 5/2007   |
| 2004/0209120 A1              | 10/2004                 | Inoue et al.      | JP | 2007-258427 A  | 10/2007  |
| 2007/0290161 A1              | 12/2007                 | Tokuoka et al.    | JP | 2007-299871 A1 | 11/2007  |
| 2008/0003126 A1              | 1/2008                  | Watanabe et al.   | JP | 2008-028162 A  | * 2/2008 |
| 2008/0012679 A1 *            | 1/2008                  | Okabe et al. .... | JP | 2008-028162 A1 | 2/2008   |
| 336/200                      |                         |                   | JP | 2008-041961 A  | * 2/2008 |
| 2008/0029300 A1              | 2/2008                  | Harada et al.     | JP | 2008-195986 A  | * 8/2008 |
| 2008/0061264 A1              | 3/2008                  | Maeda et al.      | JP | 2008-195986 A1 | 8/2008   |
| 2008/0152897 A1              | 6/2008                  | Maeda et al.      | JP | 2009-088496 A1 | 4/2009   |
| 2008/0231409 A1              | 9/2008                  | Kugai et al.      | JP | 2009-088502 A  | * 4/2009 |
| 2009/0045905 A1              | 2/2009                  | Nakagawa et al.   | JP | 2009-088502 A1 | 4/2009   |
| 2009/0102589 A1              | 4/2009                  | Lee et al.        | TW | M388724 U1     | 9/2010   |
| 2010/0253463 A1              | 10/2010                 | Shimomura et al.  | WO | 2009/128425 A1 | 10/2009  |
| 2010/0289609 A1              | 11/2010                 | Liao et al.       | WO | 2010/013843 A1 | 2/2010   |
| 2011/0024670 A1              | 2/2011                  | Otsuki et al.     |    |                |          |
| 2011/0133881 A1              | 6/2011                  | Nakajima et al.   |    |                |          |
| 2011/0227690 A1              | 9/2011                  | Watanabe et al.   |    |                |          |
| 2011/0267167 A1              | 11/2011                 | Ogawa et al.      |    |                |          |
| 2012/0038449 A1 *            | 2/2012                  | Ogawa et al. .... | JP | 2011-249774 A1 | 12/2011  |
| 336/221                      |                         |                   | JP | 2011-170349    |          |
| 2012/0070567 A1              | 3/2012                  | Watanabe et al.   |    |                |          |

**FOREIGN PATENT DOCUMENTS**

|    |                |         |
|----|----------------|---------|
| CN | 102007549 A    | 4/2011  |
| JP | H04-346204 A   | 12/1992 |
| JP | 07-201570 A    | 8/1995  |
| JP | H09-074011 A1  | 3/1997  |
| JP | 2000-030925 A1 | 1/2000  |

**OTHER PUBLICATIONS**

Non-final Office action issued by the USPTO, dated Sep. 12, 2013, for related U.S. Appl. No. 13/277,018.

Notification of Reasons for Refusal issued by the Japanese Patent Office, mailed May 29, 2013, for Japanese counterpart application No. 2011-170349.

Non-Final Rejection issued by U.S. Patent and Trademark Office, dated May 7, 2013, for related U.S. Appl. No. 13/092,381.

Office Action issued by the Korean Patent Office, mailed Nov. 4, 2013, for Korean counterpart application of a related U.S. Appl. No. 13/092,381.

\* cited by examiner

Fig. 1



Fig. 2



Fig. 3

(A)



(B)



Fig. 4



Fig. 5



Fig. 6



Fig. 7



Fig. 8



Fig. 9



Fig. 10



$$\sigma_b = \frac{M}{I} \times \frac{h}{2} = \frac{3WL}{2bh^2}$$

Width of test piece: b (mm)  
Thickness of test piece: h (mm)  
3-point bending rupture stress ( $\sigma_b$ )  
Bending moment: M  
Geometrical moment of inertia: I

Fig. 11



## 1

COIL-TYPE ELECTRONIC COMPONENT  
AND PROCESS FOR PRODUCING SAME

This application is the U.S. National Phase under 35 U.S.C. §371 of International Application PCT/JP2011/060106, filed Apr. 26, 2011, which claims priority to Japanese Patent Applications No. 2010-105552, filed Apr. 30, 2010, and No. 2011-091879, filed Apr. 18, 2011. The International Application was published under PCT Article 21(2) in a language other than English.

## TECHNICAL FIELD

The present invention relates to a coil-type electronic component and its manufacturing method. In particular, the present invention relates to a coil-type electronic component using a soft magnetic alloy suitable for coil-type electronic components that are made small enough to be mounted on the surfaces of circuit boards, as well as a manufacturing method for said coil-type electronic component.

## BACKGROUND ART

Traditionally ferrite cores, cores cut out from thin metal sheets, and compacted powder magnetic cores, are used as magnetic cores for choke coils subject to high frequencies. Metal magnetic materials provide an advantage over ferrite in that they can achieve higher saturation magnetic flux densities. On the other hand, metal magnetic materials themselves have low insulation property and must be given insulation treatment. Patent Literature 1 proposes compression-molding a mixture of Fe—Al—Si powder having surface oxide film with a binder, and then heat-treating the molded product in an oxidizing atmosphere. According to this patent literature, applying heat treatment in an oxidizing atmosphere allows for formation of an oxide layer (alumina) in areas where the insulation layer on the surface of alloy powder has broken during compression molding, thereby achieving a complex magnetic material offering good DC superimposition characteristics with small core loss. Patent Literature 2 describes a laminated electronic component whose main ingredient is metal magnetic powder, wherein said laminated electronic component is produced by stacking a metal magnetic layer formed by metal magnetic paste containing glass, with conductive patterns formed by conductive paste containing silver or other metal, thereby forming coil patterns inside the laminate, and wherein this laminated electronic component had been sintered in a nitrogen atmosphere at a temperature of 400° C. or above.

## BACKGROUND ART LITERATURE

## Patent Literature

Patent Literature 1: Japanese Patent Laid-open No. 2001-

11563

Patent Literature 2: Japanese Patent Laid-open No. 2007-27354

## SUMMARY OF THE INVENTION

## Problems to Be Solved by the Invention

The complex magnetic material described in Patent Literature 1 requires a large force at the time of compression molding because molding uses Fe—Al—Si powder having oxide film already formed on its surface. This material also presents

## 2

a problem in that it does not support further size reduction if applied to power inductors or other electronic components through which greater current must flow. The laminated electronic component described in Patent Literature 2 presents a problem in that the production cost may increase because the metal magnetic grains must be coated uniformly with glass and a nitrogen atmosphere is required to control this coating process.

The present invention was developed in light of the aforementioned situations and provides a coil-type electronic component equipped with a magnetic material that can be produced at low cost and still offers both high magnetic permeability and high saturation magnetic flux density and also provides a manufacturing process thereof.

## Means for Solving the Problems

After earnest studies repeatedly carried out to achieve the aforementioned purposes, the inventors of the present invention found that, when grains of a soft magnetic alloy containing iron, silicon and other element that oxidizes more easily than iron were mixed with a binder and the mixture was molded, and the molded product was heat-treated in an oxidizing atmosphere to break down the binder while an oxide layer was formed by oxidizing the surface of soft magnetic alloy grains, then the magnetic permeability after heat treatment would become higher when compared to the magnetic permeability before heat treatment. The inventors also found that soft magnetic alloy grains were bonded with one another, via the oxide layer, in this molded product that had been given heat treatment.

The present invention, which was completed based on the aforementioned insights, is described below: (1) A coil-type electronic component having a coil inside or on the surface of its base material, wherein said coil-type electronic component is characterized in that: the base material is constituted by a group of grains of a soft magnetic alloy (also referred to as “alloy grains” or “soft magnetic grains”) containing iron, silicon and another element that oxidizes more easily than iron; the surface of each soft magnetic alloy grain has an oxide layer formed on its surface as a result of oxidization of the grain; this oxide layer contains the other element that oxidizes more easily than iron in a quantity larger than that in the soft magnetic alloy grain; and the grains are bonded with one another via this oxide layer (2) A coil-type electronic component according to (1), characterized in that the oxide layer via which the soft magnetic grains are bonded with one another is thicker than an oxide layer other than the bonding oxide layer on the surface of the soft magnetic grains. (3) A coil-type electronic component according to (1), characterized in that the oxide layer via which the soft magnetic grains are bonded with one another is thinner than an oxide layer other than the bonding oxide layer on the surface of the soft magnetic grains. (4) A coil-type electronic component according to (1) or (2), characterized in that at least some of the soft magnetic grains are grains on which the oxide layer has a thickness of at least 50 nanometers. (5) A coil-type electronic component according to any one of (1) to (4), characterized in that the aforementioned oxide layer bonding the aforementioned grains is constituted by the same phase. (6) A coil-type electronic component according to any one of (1) to (5), characterized in that the aforementioned element that oxidizes more easily than iron is chromium. (7) A coil-type electronic component according to any one of (1) to (5), characterized in that the aforementioned element that oxidizes more easily than iron is aluminum. (8) A coil-type electronic component according to (6), characterized in that

the aforementioned soft magnetic alloy has a composition of 2 to 8 percent by weight of chromium, 1.5 to 7 percent by weight of silicon, and 88 to 96.5 percent by weight of iron. (9) A coil-type electronic component according to (7), characterized in that the aforementioned soft magnetic alloy has a composition of 2 to 8 percent by weight of aluminum, 1.5 to 12 percent by weight of silicon, and 80 to 96.5 percent by weight of iron. (10) A coil-type electronic component according to any one of (1) to (9), characterized in that the average size of the soft magnetic grains based on arithmetic mean is 30 micrometers or less. (11) A coil-type electronic component according to any one of (1) to (10), characterized in that the aforementioned oxide layer includes in this order a first oxide layer where the content of the aforementioned iron component decreases while the content of the aforementioned element that oxidizes easily increases, and a second oxide layer where the content of the aforementioned iron component decreases and the content of the aforementioned element that oxidizes easily also decreases, as viewed outwardly from the aforementioned alloy grain. (12) A coil-type electronic component according to (11), characterized in that the aforementioned first oxide layer, as viewed outwardly from the aforementioned alloy grain, has an inflection point with respect to the content of the aforementioned silicon. (13) A coil-type electronic component according to any one of (1) to (12), characterized in that the peak strength ratio of the element that oxidizes more easily than iron, relative to iron, in the oxide layer is higher than the peak strength ratio of the element that oxidizes more easily than iron, relative to iron, in the aforementioned grain, based on calculation by the ZAF method through energy diffusion X-ray analysis using a scanning electron microscope. (14) A coil-type electronic component according to any one of (1) to (13), characterized in that the aforementioned coil has its end electrically connected to a conductive film formed on the surface of the aforementioned base material. (15) A coil-type electronic component having a coil, wherein said coil-type electronic component is characterized in that: its base material is constituted by a group of grains of a soft magnetic alloy; the surface of each soft magnetic alloy grain has an oxide layer formed on its surface as a result of oxidization of the grains; this oxide layer contains a quantity of a metal that oxidizes more easily than iron, which quantity is larger than that in the alloy grains; the grains are bonded with one another via this oxide layer; and a coil conductor is formed inside this base material. (16) A coil-type electronic component according to (15), characterized in that the coil conductor forms conductive patterns and is sintered simultaneously with the base material. (17) A coil-type electronic component according to (15) or (16), characterized in that the metal that oxidizes more easily than iron in the oxide layer is chromium. (18) A coil-type electronic component according to (15) or (16), characterized in that the metal that oxidizes more easily than iron in the oxide layer is aluminum. (19) A method for manufacturing a coil-type electronic component having a coil provided in its base material, wherein said manufacturing method for a coil-type electronic component comprises: a step to press a mixture of binder and soft magnetic alloy grains to obtain a molded product; a step to heat-treat the molded product in an atmosphere containing oxygen to form an oxide layer on the surface of the soft magnetic alloy grains and bond the soft magnetic alloy grains with one another via the oxide layer to obtain a base material; and a step to provide a coil and electrodes for pulling out in the base material. (20) A method for manufacturing a coil-type electronic component having a coil provided in its base material, wherein said manufacturing method for a coil-type electronic component includes: a step

to form a mixture of binder and soft magnetic alloy grains into a sheet, form coil conductive patterns on this sheet, and stack sheets, each produced this way, on top of each other to obtain a molded product; a step to heat-treat the molded product in an atmosphere containing oxygen to form an oxide layer on the surface of the soft magnetic alloy grains and bond the soft magnetic alloy grains with one another via the oxide layer to obtain a base material having a coil inside; and a step to provide electrodes to be pulled out of the base material. (21) A manufacturing method for a coil-type electronic component according to (19) or (20), characterized in that the aforementioned oxygen atmosphere is the standard atmosphere.

#### Effects of the Invention

According to the present invention, an oxide layer formed by oxidizing each soft magnetic grain is used as an insulation layer for the grain, which makes it no longer necessary to mix resin or glass with soft magnetic grains beforehand for the purpose of insulation. There is no need, either, to apply high pressure at the time of molding compared to when Fe—Al—Si powder whose surface has been heat-treated beforehand is used. Accordingly, the present invention provides a magnetic material that can be produced at low cost and still offers both high magnetic permeability and high saturation magnetic flux density.

#### BRIEF DESCRIPTION OF THE DRAWINGS

FIG. 1 is a side view showing a first embodiment of a base material using a soft magnetic alloy for an electronic component conforming to the present invention.

FIG. 2 is an enlarged schematic section view of the base material using a soft magnetic alloy for the electronic component in the first embodiment.

FIG. 3 shows graphs indicating the results of energy diffusion X-ray analysis, using a scanning electron microscope, of the base material using a soft magnetic alloy for the electronic component in the first embodiment.

FIG. 4 shows a graph indicating the analysis results, using an X-ray diffraction analyzer, of the oxide layer of the base material using a soft magnetic alloy for the electronic component in the first embodiment.

FIG. 5 shows a graph indicating the results of linear energy diffusion X-ray analysis, using a scanning electron microscope, of the base material using a soft magnetic alloy for the electronic component in the first embodiment.

FIG. 6 is a side view, with partial perspective projection, of the first embodiment of a coil-type electronic component under the present invention.

FIG. 7 is a longitudinal section view showing the internal structure of the coil-type electronic component in the first embodiment.

FIG. 8 is a perspective view of internal structure, showing an example of variation of the embodiment of base material using a soft magnetic alloy for an electronic component conforming to the present invention.

FIG. 9 is a perspective view of internal structure, showing an example of variation of the embodiment of an electronic component under the present invention.

FIG. 10 is an explanation drawing showing how samples were measured for 3-point bending rupture stress in examples of the present invention.

FIG. 11 is an explanation drawing showing how samples were measured for volume resistivity in examples of the present invention.

## MODE FOR CARRYING OUT THE INVENTION

In the present disclosure, "an oxide layer formed as a result of oxidation of the grain" refers to an oxide layer formed by oxidation greater than natural oxidation of the grain, which oxide layer is an oxide layer grown by reacting a surface of the grain and oxygen by heat treatment of a molded body formed from grains in an oxidizing atmosphere. Also, a "layer" refers to a layer distinguishable from others based on its compositions, structures, properties, appearance, and/or production processes, etc., including a layer having a discrete or unclear boundary, and a layer which is a continuous film on the surface of a grain or which is a film having partially a discontinued portion. In some embodiments, an "oxide layer" is a continuous film covering the entire surface of each grain. Further, such an oxide layer possesses any of the characteristics identified in the present disclosure, and the oxide layer grown by oxidation of the grain surface can be distinguished from an oxide film formed by other methods. In the present disclosure, relative terms such as "greater", "easier", etc. refer to substantial differences by degrees which cause significant differences in function, structure, or effect/result. The following explains a first embodiment of a base material using a soft magnetic alloy for an electronic component conforming to the present invention, by referring to FIGS. 1 and 2. FIG. 1 is a side view showing the exterior of a base material 10 using a soft magnetic alloy for the electronic component in this embodiment. The base material 10 using a soft magnetic alloy for the electronic component in this embodiment is used as a core around which a coil of a coil-type chip inductor is wound. The core 11 has a sheet-shaped winding center 11a which is provided in parallel with the mounting surface of a circuit board, etc., and around which a coil is wound, and a pair of flange parts 11b, 11b provided at the opposing ends of the winding center 11a, which has a drum-type appearance. Coil ends are electrically connected to a conductive film 14 formed on the surface of flange parts 11b, 11b. The base material 10 using a soft magnetic alloy for the electronic component in this embodiment is constituted by a group of grains of a soft magnetic alloy containing iron (Fe), silicon (Si) and other element that oxidizes more easily than iron, characterized in that an oxide layer is formed on the surface of each soft magnetic grain through oxidization of the grain, that the oxide layer contains more chromium than does the alloy grain, and that grains are bonded with one another via this oxide layer. The descriptions below use element names or element symbols.

FIG. 2 is an enlarged schematic section view of the base material 10 using a soft magnetic alloy for the electronic component in this embodiment. The figure was created based on a composition image obtained by capturing a cross-section of the base material in its thickness direction using a SEM (scanning electron microscope) at a magnification of 3000 times. In the above schematic view, multiple grains and the oxide layer are identified as follows. First, the base material is polished until its cross-section in a thickness direction cutting across the center of the base material is exposed, and the obtained cross-section is captured with a scanning electron microscope (SEM) at a magnification of 3000 times to obtain a composition image. The scanning electron microscope (SEM) provides a composition image showing areas of different contrasts representing different constituent elements. Next, pixels of the composition image obtained above are classified into three contrast levels. The contrast ranks are determined in such a way that, among the grains shown in the above composition image whose cross-section outline can be fully observed, those whose simple average size  $D=(d_1+d_2)/2$

$d_2/2$  is greater than the average grain size ( $d_{50\%}$ ) of material grains (alloy grains having no oxide layer as an initial material), where  $d_1$  and  $d_2$  represent the long-axis dimension and short-axis dimension of the cross-section of each grain, respectively, are deemed to be of the center rank of composition contrast, and any part of the above composition image corresponding to this contrast rank is judged as a grain 1. On the other hand, any part whose composition contrast is darker than the above center contrast rank is judged as an oxide layer 2. Desirably, measurement is taken multiple times. Any part brighter than the above center contrast rank is judged as a void 3. The thickness of the oxide layer 2 can be obtained as the shortest distance from the interface between the grain and oxide layer 2 to the interface between the oxide layer 2 and the void 3.

The thickness of the oxide layer 2 is obtained specifically as follows. First, a cross-section of the base material 10 is captured in a thickness direction using an SEM (scanning electron microscope) at a magnification of 1000 to 3000 times and the center of gravity of one grain in the obtained composition image is calculated using imaging software, after which a linear analysis is conducted using an EDS (energy diffusion X-ray analyzer), starting from the center of gravity point in a radius direction. Any area whose oxygen concentration is at least three times the oxygen concentration at the center of gravity point is judged as an oxide (i.e., considering measuring errors or fluctuations, "three times" is considered to be the threshold indicating a non-oxide layer if the value is less than the threshold, and the actual oxide layer may have an oxygen concentration 100 times or more than that in the grain), and the length from this area to the outer periphery of the grain is measured as the thickness of the oxide layer 2. In some embodiments, the region of the oxide layer can be defined based on an evaluation method selected as necessary from any method disclosure in the present disclosure (distinguishing method based on brightness contrast, distinguishing method based on oxygen concentration, later-described distinguishing method based on composition, later-described distinguishing method based on peak intensity ratio, etc.), and any other conventional methods related to the presence (concentration) of oxygen. In some embodiments, the average grain size of the soft magnetic grain having an oxide layer is substantially or nearly the same as the average grain size of the material grain (grains prior to molding and heat treatment).

The thickness of the oxide layer 2 formed on the surface of the alloy grain may be caused to vary even on a single alloy grain depending on the location. In an embodiment, by bonding alloy grains, as a whole, to each other via an oxide layer thicker than the oxide layer on the surface of alloy grains (an oxide layer adjoined by a void 3), high strength can be achieved as an effect. In another embodiment, by bonding alloy grains, as a whole, to each other via an oxide layer thinner than the oxide layer on the surface of alloy grains (the oxide layer adjoined by a void 3), high magnetic permeability can be achieved as an effect. In yet another embodiment, at least some of soft magnetic grains are grains that partially have an oxide layer (as a surface oxide layer) of at least 50 nanometers in thickness. In another embodiment, the aforementioned oxide layer bonding the aforementioned grains is preferably constituted by the same phase. The "same phase" refers to a state constituted by the same crystals where respective grains are bonded continuously together via the oxide layers substantially without voids (other than voids adjoined by the oxide layers), which can be observed using a transmission electron microscope (TEM). As shown in FIG. 4, the crystalline structure can also be observed with an X-ray diffraction analyzer. The structure, composition, and thickness

of the oxide layer, as described later, can be controlled by the composition of material grains, the distance between grains (fill ratio), heat treatment temperature, heat treatment duration, oxygen content in a heat treatment atmosphere, etc. The thickness of the oxide layer varies, but in some embodiments, substantially all or most of oxide layers have a thickness of 10 to 200 nm. In another embodiment, the aforementioned oxide layer preferably includes the first oxide layer where the content of the aforementioned iron component decreases while the content of the aforementioned element that oxidizes easily increases, and the second oxide layer where the content of the aforementioned iron component decreases and the content of the aforementioned element that oxidizes easily also decreases, as viewed from the aforementioned alloy grain. It is also preferable that the aforementioned first oxide layer, as viewed from the aforementioned alloy grain, has an inflection point with respect to the content of the aforementioned silicon. The interface between the first and second oxide layers may be discrete or unclear. This structure can be observed with an EDS (energy diffusion X-ray analyzer), as shown in FIG. 5, and has the effect of keeping the saturation magnetic flux density from dropping.

The composition ratio of grains in the above base material using a soft magnetic alloy for an electronic component can be checked as follows. First, a material grain is polished until its cross-section cutting across the center of the grain is exposed, and the obtained cross-section is captured with a scanning electron microscope (SEM) at a magnification of 3000 times to obtain a composition image, which is then used to calculate the composition of  $1 \mu\text{m}^2$  near the center of the grain by the ZAF method through energy diffusion X-ray analysis (EDS). Next, the above base material using a soft magnetic alloy for an electronic component is polished until its cross-section in a thickness direction cutting across roughly the center of the base material is exposed, and the obtained cross-section is captured with a scanning electron microscope (SEM) at a magnification of 3000 times to obtain a composition image. Among the grains shown in this composition image whose cross-section outline can be fully observed, a grain is extracted, whose simple average size  $D=(d_1+d_2)/2$  is greater than the average grain size of material grains (d50%), where  $d_1$  and  $d_2$  represent the long-axis dimension and short-axis dimension of the cross-section of each grain, respectively, and the composition of  $1 \mu\text{m}^2$  near the point of intersection of its long axis and short axis is calculated by the ZAF method through energy diffusion X-ray analysis (EDS). The result is then compared against the composition ratio in the above material grain to show the composition ratio in the alloy grain of the above base material using a soft magnetic alloy for an electronic component. (Since the composition of the material grain is known, by comparing the composition ratios determined by the ZAF method, the composition of the alloy grain can be determined.) The thickness of the oxide layer on the above base material using a soft magnetic alloy for an electronic component was determined as the average thickness  $T=(t_1+t_2)/2$ , where  $t_1$  represents the thickness of the oxide layer present on the surface of grains 1, 1 identified by the above method, measured at the thickest part farthest away from the grain 1, while  $t_2$  represents the thickness at the thinnest part.

An embodiment of the present invention is explained using an example where the element that oxidizes easily is chromium. The base material 10 using a soft magnetic alloy for the electronic component in this embodiment has multiple grains 1, 1 each containing 2 to 8 percent by weight of chromium, 1.5 to 7 percent by weight of silicon, and 88 to 96.5 percent by weight of iron, and an oxide layer 2 generated on the surface

of each grain 1. The oxide layer 2 contains at least iron and chromium, where the peak strength ratio R2 of chromium relative to iron, as measured by energy diffusion X-ray analysis using a transmission electron microscope, is substantially greater than the peak strength ratio R1 of chromium relative to iron in the grain. (For example, R2 is at least several times or several tens of times greater than R1.) There are also voids 3 between multiple grains. In the above base material using a soft magnetic alloy for the electronic component, the peak strength ratio R2 of chromium relative to iron in the above oxide layer 2, and strength ratio R1 of chromium relative to iron in the above grain 1, can be respectively obtained as follows. First, SEM-EDS analysis is performed on the above composition image to obtain the composition of  $1 \mu\text{m}^2$  around the point of intersection of the long axis  $d_1$  and short axis  $d_2$  inside the grain 1. Next, SEM-EDS analysis is performed on the above composition image to obtain the composition of  $1 \mu\text{m}^2$  around the center point of the oxide layer in a thickness direction in the location where the thickness of the oxide layer corresponds to the average thickness  $T=(t_1+t_2)/2$ , where  $t_1$  represents the thickness of the oxide layer 2 on the surface of the grain 1 as measured at the thickest part, while  $t_2$  represents the thickness at the thinnest part. Now, the peak strength of chromium relative to iron, or  $R1=C_{1\text{CrKa}}/C_{1\text{FeKa}}$ , can be obtained from the strength of iron, or  $C_{1\text{FeKa}}$ , and strength of chromium, or  $C_{1\text{CrKa}}$ , in the grain 1. Also, the peak strength of chromium relative to iron, or  $R2=C_{2\text{CrKa}}/C_{2\text{FeKa}}$ , can be obtained from the strength of iron, or  $C_{2\text{FeKa}}$ , and strength of chromium, or  $C_{2\text{CrKa}}$ , at the center point of the oxide layer 2 in a thickness direction.

Also, with the base material using a soft magnetic alloy for an electronic component as proposed by the present invention, bonding of adjacent grains 1, 1 via an oxide layer formed on their surface can be confirmed by a schematic drawing, like the one shown in FIG. 2, created from the above composition image. This bonding of adjacent grains 1, 1 via an oxide layer formed on their surface also manifests as improved magnetic characteristics and strength of the base material using a soft magnetic alloy for an electronic component.

To manufacture the base material using a soft magnetic alloy for an electronic component as proposed by the present invention, one embodiment is that first a binder such as a thermoplastic resin or the like is added to material grains containing chromium, silicon and iron, and the mixture is agitated and kneaded to obtain pellets. Next, these pellets are compression-molded to form a molded product, and the obtained molded product is heat-treated at 400 to 900°C. in the standard atmosphere. This heat treatment in the standard atmosphere degreases the thermoplastic resin that has been mixed in, generates an oxide layer constituted by metal oxide on the grain surface while bonding chromium that was present in the grain and has migrated to the surface as a result of heat treatment, with iron and oxygen that are main ingredients of the grain, and also bonds the oxide layers on the surface of adjacent grains. The generated oxide layer (layer of metal oxide) is an oxide constituted primarily by Fe and Cr, which ensures insulation between grains to help provide a base material using a soft magnetic alloy for the electronic component. Material grains may be those manufactured by the water atomization method, for example, and material grains may have a spherical or flat shape, among others.

Under the present invention, raising the heat treatment temperature in an oxygen atmosphere causes the binder to break down and the soft magnetic alloy to be oxidized. Accordingly, desirable heat treatment conditions for the molded product are such that a temperature between 400 and 900°C. is held for at least 1 minute in the standard atmo-

sphere. As long as heat treatment is applied within this temperature range, an excellent oxide layer can be formed. A more preferable temperature range is 600 to 800° C. Heat treatment may be performed in a condition other than the standard atmosphere, such as in an atmosphere where the oxygen component pressure is equivalent to that in the standard atmosphere. In a reducing atmosphere or non-oxidizing atmosphere, an oxide layer constituted by metal oxide is not formed by heat treatment, resulting in sintering of grains and significant drop in volume resistivity. The oxygen concentration and amount of steam in an atmosphere are not specifically limited, but desirably the standard atmosphere or dry air is used from the viewpoint of production. When the heat treatment temperature exceeds 400° C., excellent strength and excellent volume resistivity can be obtained. If the heat treatment temperature exceeds 900° C., on the other hand, the strength will increase but the volume resistivity will drop. Holding the heat treatment temperature mentioned above for at least 1 minute facilitates the generation of an oxide layer constituted by a metal oxide containing Fe and Cr. Since the thickness of the oxide layer saturates at a specific value, the maximum holding time is intentionally not set. However, 2 hours or less is appropriate in consideration of productivity. As explained above, a base material using a soft magnetic alloy with an oxide layer, which offers both excellent strength and excellent volume resistivity, can be obtained by adjusting the heat treatment conditions within the above ranges. In other words, the heat treatment temperature, heat treatment time, oxygen content in the heat treatment atmosphere, etc. are used to control the formation of an oxide layer.

With the base material using a soft magnetic alloy for an electronic component as proposed by the present invention, the above treatment is applied to alloy powder constituted by iron, silicon and other element that oxidizes more easily than iron, to achieve high magnetic permeability and high saturation magnetic flux density. Due to this high magnetic permeability, electronic components through which greater current can flow are obtained with a smaller base material using a soft magnetic alloy when compared to the conventional ones. Unlike a coil device wherein soft magnetic alloy grains are bonded using resin or glass, since neither resin nor glass is used, and application of high pressure is not necessary during molding, low-cost production is possible. Also with the base material using a soft magnetic alloy for the electronic component in this embodiment, high saturation magnetic flux density is maintained and even after the heat treatment in the standard atmosphere, glass component, etc., will not migrate to the surface of the base material and thus small chip electronic components that offer high dimensional stability can be provided.

Next, the first embodiment of an electronic component conforming to the present invention is explained by referring to FIGS. 1, 2, 6 and 7. FIGS. 1 and 2 are not explained here, because they were already explained in connection with the earlier embodiment of base material using a soft magnetic alloy for an electronic component. FIG. 6 is a side view, with partial perspective projection, of the electronic component in this embodiment. FIG. 7 is a longitudinal section view showing the internal structure of the electronic component in this embodiment. The electronic component 20 in this embodiment is a coil-type electronic component, or specifically a winding-type chip inductor. It is comprised of a drum-type core 11 constituting the above base material 10 using a soft magnetic alloy for an electronic component, and the aforementioned base material 10, and has a pair of sheet-shaped cores 12, 12, which are not illustrated, connecting the two flange parts 11b, 11b of the drum-type core 11. On the instal-

lation surfaces of the flange parts 11, 11b of the core 11, a pair of external conductive films 14, 14 are formed, respectively. Also, a coil 15 constituted by an insulation coated conductive wire is wound around the winding center 11a of the core 11 to form a winding part 15a, while both ends 15b, 15b are thermo-compression-bonded to the external conductive films 14, 14 on the installation surfaces of the flange parts 11b, 11b, respectively. The external conductive films 14, 14 each have a baked conductive layer 14a formed on the surface of the base material 10, as well as a Ni plating layer 14b and Sn plating layer 14c that are layered on top this baked conductive layer 14a. The aforementioned sheet-shaped cores 12, 12 are bonded by resin adhesive to the flange parts 11b, 11b of the drum-type core 11.

The electronic component 20 in this embodiment has: multiple grains containing chromium, silicon and iron; an oxide layer formed on the surface of these grains, wherein this oxide layer contains at least iron and chromium and whose peak strength ratio of chromium relative to iron is higher than the peak strength ratio of chromium relative to iron in the aforementioned grain, based on calculation by the ZAF method through energy diffusion X-ray analysis using a scanning electron microscope; and a base material 10, as a core 11, which uses the aforementioned soft magnetic alloy for an electronic component where oxide layers formed on the surfaces of the aforementioned grains adjacent to one another are bonded. At least a pair of external conductive layers 14, 14 are formed on the surface of the base material 10. The base material 10 using a soft magnetic alloy for the electronic component, which constitutes the electronic component 20 in this embodiment, is not explained here because it has already been explained earlier.

The core 11 at least has a winding center 11a, where the cross-section of the winding center 11a may be sheet-shaped (rectangular), circular or oval. Also, it is desirable that at least one flange part 11 is provided on one end of the aforementioned winding center 11a. With a flange part 11, the coil position relative to the winding center 11a can be controlled easily using the flange part 11, to help stabilize characteristics such as inductance and the like. The core 11 can be embodied in several ways, such as an embodiment with one flange part, embodiment with two flange parts (drum core), embodiment where the long-axis direction of the winding center 11a is placed vertically to the installation surface, and embodiment where the long-axis direction is placed horizontally to the installation surface. Especially, an embodiment where a flange part is provided only on one axial end of the winding center 11a and the long-axis direction of the winding center 11a is placed vertically to the installation surface, is preferable in reducing the height.

The conductive film 14 is formed on the surface of the base material 10 using a soft magnetic alloy for an electronic component, and an end of the coil is connected to the conductive film 14. The conductive film 14 may be a baked conductive film or resin conductive film. A baked conductive film can be formed on the base material 10 using a soft magnetic alloy for an electronic component by, for example, baking a paste made of silver to which glass has been added at a specified temperature. A resin conductive film can be formed on the base material 10 using a soft magnetic alloy for an electronic component by, for example, applying a paste containing silver and epoxy resin and then treating the paste at a specified temperature. In the case of baked conductive film, heat treatment can be applied after the conductive film has been formed.

The coil may be made of copper or silver. Desirably the coil is given insulation coating. The coil may be a rectangular

wire, angular wire, or rounded wire. Use of a rectangular or angular wire is desirable because the gaps between windings can be reduced and the electronic component can be kept small.

A specific example of forming the baked conductive layer 14a that constitutes the conductive films 14, 14 on the surface of the base material 10 using a soft magnetic alloy for an electronic component in the electronic component 20 in this embodiment, is given below. Bake-type electrode material paste containing metal grains and glass frit (bake-type Ag paste is used in this example) is applied on the installation surfaces of the flange parts 11b, 11b of the base material 10, or core 11, and then heat treatment is given in the standard atmosphere to sinter and affix the electrode material directly on the surface of the base material 10. Ni and Sn metal plating layers may also be formed, by means of electrolysis, on the surface of the baked conductive layer 14a that has been formed.

The electronic component 20 in this embodiment can also be obtained by the manufacturing method explained below. Material containing material grains and binder is molded, where the specific composition of material grains is, say, 2 to 8 percent by weight of chromium, 1.5 to 7 percent by weight of silicon and 88 to 96.5 percent by weight of iron, and bake-type electrode material paste containing metal powder and glass frit is applied on the surface of the obtained molded product at least over an area that will become the installation surface, and the resulting molded product is heat-treated at 400 to 900° C. in the standard atmosphere. Metal plating layers may also be formed on the baked conductive layer that has been formed. According to this method, an oxide layer is generated on the surface of grains, and a base material using a soft magnetic alloy for an electronic component where oxide layers on the surfaces of adjacent grains are bonded with one another can be formed simultaneously with a baked conductive layer constituting the conductive film on the surface of this base material, which simplifies the manufacturing process. Since chromium oxidizes more easily than iron, excessive oxidization of iron can be prevented when heat is applied in an oxidizing atmosphere, compared to pure iron. Other than chromium, aluminum can also be used.

Next, an example of variation of the embodiment of the base material using a soft magnetic alloy for an electronic component under the present invention is explained by referring to FIG. 8. FIG. 8 is a perspective view of internal structure, showing an example of variation of the base material 10' using a soft magnetic alloy for an electronic component. The base material 10' in this example of variation has a rectangular solid appearance, while on the inside an internal coil 35 wound in helical manner is buried and the pullout parts at both ends of the internal coil 35 are exposed to a pair of opposing end faces of the base material 10'. The base material 10', together with the internal coil 35 buried inside, constitutes a laminated chip 31. Just like the base material 10 using a soft magnetic alloy for the electronic component in the first embodiment described earlier, the base material 10' using a soft magnetic alloy for the electronic component in this example of variation is also characterized in that it has: multiple grains containing chromium, silicon and iron; an oxide layer formed on the surface of these grains, wherein this oxide layer contains at least iron and chromium and whose peak strength ratio of chromium relative to iron is higher than the peak strength ratio of chromium relative to iron in the grain, based on energy diffusion X-ray analysis using a scanning electron microscope, and wherein oxide layers formed on the surfaces of adjacent grains are bonded with one another. The base material 10' using a soft magnetic alloy for the electronic

component in this example of variation also has the same operations and effects as those of the base material 10 using a soft magnetic alloy for the electronic component in the first embodiment described earlier.

Next, an example of variation of the embodiment of an electronic component under the present invention is explained by referring to FIG. 9. FIG. 9 is a perspective view of internal structure, showing an electronic component 40 being an example of variation. The electronic component 40 in this example of variation is constituted by the base material 10' using a soft magnetic alloy for the electronic component described in the aforementioned example of variation, where a pair of external conductive films 34, 34 are formed on or near a pair of opposing end faces of the base material in a manner connecting the exposed pullout parts of the internal coil 35. These external conductive films 34, 34, while not illustrated, have a baked conductive layer and an Ni plating layer and an Sn plating layer that are layered on top of this baked conductive layer, just like the external conductive layers 14, 14 of the electronic component 20 in the first embodiment described earlier.

In addition, it is desirable that the multiple grains constituting the base material using a soft magnetic alloy for an electronic component, as proposed by the present invention, should have a composition of "2 percent by weight≤Chromium≤8 percent by weight," "1.5 percent by weight≤Silicon≤7 percent by weight" and "88 percent by weight≤Iron≤96.5 percent by weight." When the respective components are within these ranges, the base material using a soft magnetic alloy for an electronic component as proposed by the present invention demonstrates even higher strength and higher volume resistivity. In general, soft magnetic alloys containing larger amounts of Fe have higher saturation magnetic flux densities and thereby offering better DC superimposition characteristics. However, higher Fe contents mean generation of rust in a condition of high temperature and humidity, which causes various problems in use, such as shedding of rusted material. It is a well-known fact that adding chromium to magnetic alloys is effective in raising the corrosion resistance of alloys, one representative example of which is stainless steel. However, when compacted powder magnetic cores were made from such magnetic alloy powder containing chromium by applying heat treatment in a non-oxidizing atmosphere, specific resistances measured by an insulation resistance tester were around  $10^{-1}$  Ωcm, which is enough to prevent eddy-current loss between grains, but short of  $10^5$  Ωcm or more needed to form an external conductive film, and as a result no metal plating layer could be formed on the baked conductive layer constituting the external conductive film.

Accordingly, under the present invention, a molded product containing a binder and material grains having the aforementioned composition is heat-treated in an oxidizing atmosphere to generate on the surface of grains an oxide layer constituted by a metal oxide layer, while causing oxide layers on the surfaces of adjacent grains to be bonded with one another, to achieve high strength. The base material using a soft magnetic alloy for an electronic component, thus obtained, had a greatly improved volume resistivity  $\rho_v$  of  $10^5$  Ωcm or more, which made it possible to form plating layers of metal such as Ni, Sn and the like, without causing plating extension, on the baked conductive layer constituting the external conductive film formed on the surface of the base material.

The reason the composition is limited for the base material using a soft magnetic alloy for an electronic component, in a more favorable form of the present invention, is explained. If

## 13

the chromium content in the composition of multiple grains is less than 2 percent by weight, the volume resistivity becomes low and no metal plating layer can be formed, without causing plating extension, on the baked conductive layer constituting the external conductive film.

If chromium is contained by more than 8 percent by weight, the volume resistivity also becomes low and no metal plating layer can be formed, without causing plating extension, on the baked conductive layer constituting the external conductive film. If an oxide coat is formed using Fe—Si—Al powder via heat treatment in the standard atmosphere, as described in Patent Literature 1 above, the coat is constituted by a chromium-free oxide. As a result, its volume resistivity becomes lower than  $10^5 \Omega\text{cm}$  and no metal plating layer can be formed, without causing plating extension, on the baked conductive layer constituting the external conductive film.

With the above base material using a soft magnetic alloy for an electronic component, Si in the composition of multiple grains has the effect of improving the volume resistivity, but this effect is not achieved when the content is less than 1.5 percent by weight, while the achieved effect is not sufficient when the content is more than 7 percent by weight, and the volume resistivity is also less than  $10^5 \Omega\text{cm}$ , which means that no metal plating layer can be formed, without causing plating extension, on the baked conductive layer constituting the external conductive film. Si also has the effect of improving the magnetic permeability, but if the content is more than 7 percent by weight, a relative decrease in Fe content causes the saturation magnetic flux density to drop. It also results in lower moldability, which is another factor that lowers the magnetic permeability and the saturation magnetic flux density.

If aluminum is used as the element that oxidizes easily, instead of chromium, a desirable composition is 2 to 8 percent by weight of aluminum, 1.5 to 12 percent by weight of silicon, and 80 to 96.5 percent by weight of iron. If the aluminum content in the composition of multiple grains is less than 2 percent by weight, the volume resistivity becomes low and no metal plating layer can be formed, without causing plating extension, on the baked conductive layer constituting the external conductive film. If the aluminum content is more than 8 percent by weight, on the other hand, a relative decrease in Fe content causes the saturation magnetic flux density to drop. From the viewpoint of rust-resistance, a desirable composition is 2 to 8 percent by weight of chromium, 1.5 to 7 percent by weight of silicon, and 88 to 96.5 percent by weight of iron. It is also possible to mix grains of an alloy of iron, chromium and silicon, with grains of an alloy of iron, aluminum and silicon (in an amount, for example, of less than 50% by weight of the total alloy grains).

With the above base material using a soft magnetic alloy for an electronic component, the saturation magnetic flux density drops, while moldability also drops to decrease the magnetic permeability and saturation magnetic flux density, if the iron content in the composition of multiple grains is less than 88 percent by weight. If the iron content is more than 96.5 percent by weight, the volume resistivity drops due to a relative drop in chromium content and silicon content.

Under the present invention, it is also desirable that the average size of multiple grains is 5 to 30  $\mu\text{m}$  in equivalent average grain size  $d_{50\%}$  (arithmetic mean) of material grains. Also note that the average size of multiple grains mentioned above can be approximated by a value obtained by capturing a composition image of a cross-section of the base material using a scanning electron microscope (SEM) at a magnification of 3000 times, and then dividing the total sum of simple averages  $D=(d_1+d_2)/2$  of grains whose cross-section outline

## 14

can be fully observed, by the total number of grains, where  $d_1$  and  $d_2$  represent the long-axis dimension and short-axis dimension of the cross-section of each grain, respectively.

The group of alloy metal grains has a granular distribution, and grains are not necessarily circular but have irregular shapes instead. When solid alloy metal grains are observed two-dimensionally (on a plane), their size varies depending on which cross-section is observed. Accordingly, under the present invention, the average grain size is evaluated by measuring more grains. In this sense, it is desirable to measure at least 100 applicable grains under the conditions specified below. The specific method is as follows. First the largest diameter of the grain cross-section represents the long axis, and the point that equally divides the length of the long axis is obtained. Next, the smallest diameter of the grain cross-section that includes this point represents the short axis. The two are defined as the long-axis dimension and short-axis dimension, respectively. Grains to be measured are arranged sequentially from the one having the largest diameter of its cross-section, and measurement is performed until the cumulative ratio of grain cross-sections accounts for 95% of all area shown in the scanning electron microscope (SEM) image excluding grains whose cross-section outline is cannot be fully observed, voids, and oxide layers. As long as the average grain size mentioned above is within the specified range, high saturation magnetic flux density (1.4 T or more) and high magnetic permeability (27 or more) can be obtained, and generation of eddy-current loss in the grain can be prevented even at frequencies of 100 kHz and above. In the present disclosure, disclosed numeral numbers refer to approximate numbers in some embodiments, and the upper and lower endpoints of described ranges are included in some embodiments, or excluded in some embodiments. Further, in some embodiments, numeral numbers refer to average numbers, representative numbers, median, etc.

## EXAMPLES

The following explains the present invention in greater detail using examples and a comparative example. It should be noted, however, that the present invention is not at all limited to these examples and the comparative example.

To determine the level of magnetic characteristics of each base material using a soft magnetic alloy for an electronic component, grain materials were molded into a toroidal shape of 14 mm in outer diameter, 8 mm in inner diameter and 3 mm in thickness by adjusting the molding pressure to between 6 and 12 tons/cm<sup>2</sup> so that the fill ratio of material grains would become 80 percent by volume, after which the molded product was heat-treated in the standard atmosphere and a coil constituted by urethane-coated copper wire of 0.3 mm in diameter was wound around the obtained base material by 20 turns to obtain a test sample. Saturation magnetic flux density  $B_s$  was measured with a vibration sample magnetometer (VSM manufactured by Toei Industry), while magnetic permeability  $\mu$  was measured with an L chromium meter (4285A manufactured by Agilent Technologies) at a measurement frequency of 100 kHz. Samples whose saturation magnetic flux density  $B_s$  was 0.7 T or more were considered of good quality. Samples whose magnetic permeability  $\mu$  was 20 or more were considered of good quality.

To determine the level of strength of each base material using a soft magnetic alloy for an electronic component, 3-point bending rupture stress was measured, as follows, according to the measurement method illustrated in FIG. 10. Each test piece used for measurement of 3-point bending rupture stress was prepared by molding material grains into a

sheet shape of 50 mm in length, 10 mm in width and 4 mm in thickness by adjusting the molding pressure to between 6 and 12 tons/cm<sup>2</sup> so that the fill ratio of material grains would become 80 percent by volume, and then heat-treating the molded product in the standard atmosphere. Samples whose 3-point bending rupture stress was 1.0 kgf/mm<sup>2</sup> or more were considered of good quality. Overall, samples whose saturation magnetic flux density  $B_s$ , magnetic permeability  $\mu$  and 3-point bending rupture stress were all of good quality, were considered acceptable.

In addition, to determine the level of volume resistivity of each base material using a soft magnetic alloy for an electronic component, measurement was performed, as shown in FIG. 11, according to JIS-K6911. Each test piece used for measurement of volume resistivity was prepared by molding material grains into a disk shape of 100 mm in diameter and 2 mm in thickness by adjusting the molding pressure to between 6 and 12 tons/cm<sup>2</sup> so that the fill ratio of material grains would become 80 percent by volume, and then heat-treating the molded product in the standard atmosphere. Samples whose volume resistivity was  $1 \times 10^{-3} \Omega\text{cm}$  or more were considered of acceptable quality,  $1 \times 10^{-1} \Omega\text{cm}$  or more of good quality, and  $1 \times 10^5 \Omega\text{cm}$  or more of excellent quality. As long as the volume resistivity is  $1 \times 10^{-1} \Omega\text{cm}$  or more, loss due to eddy current can be kept small when used at high frequencies. If the volume resistivity is  $1 \times 10^5 \Omega\text{cm}$  or more, metal plating layers can be formed on top of the conductive layer by wet plating.

Furthermore, to determine the level of formability of metal plating layers on the baked conductive layer constituting the external conductive film on the surface of the base material using a soft magnetic alloy for an electronic component, a drum-type base material is used in the following examples for the base material using a soft magnetic alloy for an electronic component, in terms of the base material shape. To determine the level of formability of metal plating layers on the external conductive film on the obtained electronic component sample, appearance of samples was visually examined using a magnifying glass and those having Ni and Sn plating layers formed continuously on the baked conductive layer without the plating extending from the baked conductive layer into surrounding areas were considered acceptable (O), and others were considered unacceptable (X).

#### Example 1

For the material grains to obtain a base material using a soft magnetic alloy for an electronic component, alloy powder (PF-20F manufactured by Epson Atmix K.K.) was used which is a type of water-atomized powder whose average grain size (d50%) is 10 $\mu$  and composition ratio was 5 percent by weight of chromium, 3 percent by weight of silicon and 92 percent by weight of iron. The average grain size d50% of material grains described above was measured using a granularity analyzer (9320HRA manufactured by Nikkiso). Each of the above grains was polished until its cross-section in a thickness direction cutting across roughly the center of the grain was exposed, and the obtained cross-section was captured with a scanning electron microscope (SEM: S-4300SE/N manufactured by Hitachi High-Technologies) at a magnification of 3000 times to obtain a composition image, which was then used to calculate the composition of 1  $\mu\text{m}^2$  near the center of the grain and also near the surface by the ZAF method through energy diffusion X-ray analysis (EDS), confirming that the above composition ratio near the center of the grain was roughly the same as the corresponding composition ratio near the surface. Next, the above grains were

mixed with polyvinyl butylal (S-LEC BL, a solution with a solid concentration of 30 percent by weight, manufactured by Sekisui Chemical) using a wet-type rolling agitator to obtain pellets. The obtained pellets were molded into an angular sheet shape of 50 mm in length, 10 mm in width and 4 mm in thickness; a disk shape of 100 mm in diameter and 2 mm in thickness; a toroidal shape of 14 mm in outer diameter, 8 mm in inner diameter and 3 mm in thickness; a drum-type core having angular flange parts (1.6 mm wide $\times$ 0.6 mm high $\times$ 0.3 mm thick) at both ends of winding core parts (1.0 mm wide $\times$ 0.36 mm high,  $\times$ 1.4 mm long); and a pair of sheet-shaped cores (2.0 mm long $\times$ 0.5 mm wide,  $\times$ 0.2 mm thick), by adjusting the molding pressure to between 6 and 12 tons/cm<sup>2</sup> so that the fill ratio of multiple grains would become 80 percent by volume. The disk-shaped molded product, toroidal molded product, drum-type molded product and pair of sheet-shaped molded products, as obtained above, were heat-treated at 700°C. for 60 minutes in the standard atmosphere.

The disk-shaped base material obtained by heat-treating the above disk-shaped molded product was measured for volume resistivity according to JIS-K6911, and the result is shown in Table 1. Also, the drum-type base material obtained by heat-treating the above drum-type molded product was polished until its cross-section in thickness direction cutting across roughly the center of the winding center was exposed, and the obtained cross-section was captured with a scanning electron microscope (SEM) at a magnification of 3000 times to obtain a composition image. Next, pixels of the composition image obtained above were classified into three contrast levels. The contrast ranks were determined in such a way that, among the grains shown in the above composition image whose cross-section outline could be fully observed, those whose simple average size  $D=(d_1+d_2)/2$  was greater than the average grain size of material grains (d50%), where d1 and d2 represent the long-axis dimension and short-axis dimension of the cross-section of each grain, respectively, were deemed to be of the center rank of composition contrast, and any part of the above composition image corresponding to this contrast rank was judged as a grain 1. On the other hand, any part whose composition contrast was darker than the above center contrast rank was judged as an oxide layer 2. In addition, any part brighter than the above center contrast rank was judged as a void 3. The obtained result is shown by a schematic drawing in FIG. 2.

Next, among the grains shown in this composition image whose cross-section outline could be fully observed, a grain whose simple average size  $D=(d_1+d_2)/2$  was greater than the average grain size of material grains (d50%), where d1 and d2 represent the long-axis dimension and short-axis dimension of the cross-section of each grain, respectively, was extracted and the composition of 1  $\mu\text{m}^2$  near the point of intersection of its long axis and short axis was calculated by the ZAF method through energy diffusion X-ray analysis (EDS). The result was then compared against the composition ratio of the above material grain to confirm that the composition ratio of multiple grains constituting the above base material was roughly or substantially the same as the composition ratio of material grains.

Next, SEM-EDS analysis was performed on the above composition image to obtain the composition of 1  $\mu\text{m}^2$  around the point of intersection of the long axis d1 and short axis d2 inside the grain 1, and the result is shown in FIG. 3 (A). Then, SEM-EDS analysis was performed on the above composition image to obtain the composition of 1  $\mu\text{m}^2$  around the center point of the oxide layer in a thickness direction in the location where the thickness of the oxide layer corresponded to the average thickness  $T=(t_1+t_2)/2$ , where t1

represents the thickness of the oxide layer 2 on the surface of the grain 1 as measured at the thickest part, while  $t_2$  represents the thickness at the thinnest part, and the result is shown in FIG. 3 (B). From FIG. 3 (A), the strength of iron in the grain 1, or  $C1_{FeKa}$ , is 4200 count, the strength of chromium  $C1_{CrKa}$  is 100 count, and the peak strength ratio of chromium relative to iron, or  $R1=C1_{CrKa}/C1_{FeKa}$ , is 0.024. From FIG. 3 (B), the strength of iron at the center point of the oxide layer 2 in a thickness direction, or  $C2_{FeKa}$ , is 3000 count, the strength of chromium  $C2_{CrKa}$  is 1800 count, and the peak strength ratio of chromium relative to iron, or  $R2=C2_{CrKa}/C2_{FeKa}$ , is 0.60, which is higher than  $R1$  indicating the peak strength ratio of chromium relative to iron in the aforementioned grain. Also with the base material using a soft magnetic alloy for an electronic component under the present invention, it could be confirmed from the schematic drawing in FIG. 2 derived from the above composition image, that oxide layers 2, 2 formed on the surfaces of adjacent grains 1, 1 were bonded with one another.

The above results confirmed that the base material using a soft magnetic alloy for an electronic component in Example 1 had multiple grains 1, 1 containing 2 to 8 percent by weight of chromium, 1.5 to 7 percent by weight of silicon and 88 to 96.5 percent by weight of iron, and an oxide layer generated on the surface of each grain 1, wherein the oxide layer contained at least iron and chromium and its peak strength ratio of chromium relative to iron was higher than the peak strength ratio of chromium relative to iron in the grain, based on energy diffusion X-ray analysis using a transmission electron microscope. In addition, a coil constituted by urethane-coated copper wire of 0.3 mm in diameter was wound by 20 turns around the toroidal base material obtained by heat-treating the above toroidal molded product, to obtain a test sample. Saturation magnetic flux density  $B_s$  was measured with a vibration sample magnetometer (VSM manufactured by Toei Industry), while magnetic permeability  $\mu$  was measured with an LCR meter (4285A manufactured by Agilent Technologies) at a measurement frequency of 100 kHz. The obtained results are shown in Table 1.

Furthermore, the angular sheet-shaped molded product obtained above was heat-treated in the standard atmosphere for 60 minutes at 150°C., 200°C., 300°C., 500°C., 600°C., 700°C., 800°C. and 1000°C., respectively, and then the obtained angular sheet-shaped base materials, as well as angular sheet-shaped molded product that was let to stand at room temperature, were measured for 3-point bending rupture stress. The results are shown in Tables 1 and 2. Also, bake-type Ag conductive film paste was applied on the installation surfaces of the two flange parts of the above drum-type base material, after which the conductive film material was baked by heating up to 700°C. in the standard atmosphere over a period of approx. 30 minutes, holding at 700°C. for 10 minutes, and then lowering the temperature over a period of 30 minutes, to form a baked conductive layer constituting an external conductive film. This was followed by formation of Ni (2 µm in thickness) and Sn (7 µm in thickness) on the surface of this conductive film via the electrolytic plating method.

The obtained results are shown in Table 1. All of the results of measurement and judgment were favorable, with the strength of the base material being 7.4 kgf/mm<sup>2</sup>, magnetic characteristics being 1.51 T in saturation magnetic flux density  $B_s$  and 45 in magnetic permeability  $\mu$ , volume resistivity being  $4.2 \times 10^5$  Ωcm, and formability of metal plating layer being 0. Note that magnetic permeability  $\mu$  was also measured before the heat treatment. The result is shown in Table 3. Next, a coil constituted by insulation-coated conductive wire

was wound around the winding center of the above drum-type base material and both ends were thermo-compression-bonded to the above external conductive film, respectively, after which the base material obtained by heat-treating the above sheet-shaped molded product was bonded via resin adhesive to both sides of the flange parts of the above drum-type base material, to obtain a winding-type chip inductor.

#### Example 2

Evaluation samples were created in the same manner as in Example 1, except that the composition ratio of material grains was changed to 3 percent by weight of chromium, 5 percent by weight of silicon and 92 percent by weight of iron. The obtained results are shown in Tables 1 and 2. As shown in Tables 1 and 2, all of the results of measurement and judgment were favorable, as in Example 1, with the magnetic characteristics being 1.46 T in saturation magnetic flux density  $B_s$  and 43 in magnetic permeability  $\mu$ , strength of the base material being 2.8 kgf/mm<sup>2</sup>, volume resistivity being  $2.0 \times 10^5$  Ωcm, and formability of metal plating layer being 0. SEM-EDS analysis confirmed that the grains were bonded with one another via the metal oxide (oxide layer) formed on the surfaces of the grains by the heat treatment, and the oxide layer was an oxide containing an element that oxidizes more easily than iron (here chromium) by a quantity larger than that in the alloy grains.

#### Example 3

Evaluation samples were created in the same manner as in Example 1, except that the average grain size (d50%) of material grains was changed to 6 µm. The obtained results are shown in Tables 1 and 2. As shown in Tables 1 and 2, all of the results of measurement and judgment were favorable, as in Example 1, with the magnetic characteristics being 1.45 T in saturation magnetic flux density  $B_s$  and 27 in magnetic permeability  $\mu$ , strength of the base material being 6.6 kgf/mm<sup>2</sup>, volume resistivity being  $3.0 \times 10^5$  Ωcm, and formability of metal plating layer being 0. SEM-EDS analysis confirmed that the grains were bonded with one another via the metal oxide (oxide layer) formed on the surfaces of the grains by the heat treatment, and the oxide layer was an oxide containing an element that oxidizes more easily than iron (here chromium) by a quantity larger than that in the alloy grains.

#### Example 4

Evaluation samples were created in the same manner as in Example 1, except that the average grain size (d50%) of material grains was changed to 3 µm. The obtained results are shown in Tables 1 and 2. As shown in Tables 1 and 2, all of the results of measurement and judgment were favorable, as in Example 1, with the magnetic characteristics being 1.38 T in saturation magnetic flux density  $B_s$  and 20 in magnetic permeability  $\mu$ , strength of the base material being 7.6 kgf/mm<sup>2</sup>, volume resistivity being  $7.0 \times 10^5$  Ωcm, and formability of metal plating layer being 0. SEM-EDS analysis confirmed that the grains were bonded with one another via the metal oxide (oxide layer) formed on the surfaces of the grains by the heat treatment, and the oxide layer was an oxide containing an element that oxidizes more easily than iron (here chromium) by a quantity larger than that in the alloy grains.

#### Example 5

Evaluation samples were created in the same manner as in Example 1, except that the composition ratio of material

19

grains was changed to 9.5 percent by weight of chromium, 3 percent by weight of silicon and 87.5 percent by weight of iron. The obtained results of measurement and judgment are shown in Tables 1 and 2. As shown in Tables 1 and 2, the magnetic characteristics were 1.36 T in saturation magnetic flux density  $B_s$  and 33 in magnetic permeability  $\mu$ , strength of the base material was 7.4 kgf/mm<sup>2</sup>, volume resistivity was  $4.7 \times 10^{-3}$   $\Omega$ cm, and formability of metal plating layer was X. From this example, it was found that the volume resistivity would drop if the chromium content exceeds 8 percent by weight. SEM-EDS analysis confirmed that the grains were bonded with one another via the metal oxide (oxide layer) formed on the surfaces of the grains by the heat treatment, and the oxide layer was an oxide containing an element that oxidizes more easily than iron (here chromium) by a quantity larger than that in the alloy grains.

#### Example 6

Evaluation samples were created in the same manner as in Example 1, except that the composition ratio of material grains was changed to 5 percent by weight of chromium, 1 percent by weight of silicon and 94 percent by weight of iron. The obtained results of measurement and judgment are shown in Tables 1 and 2. As shown in Tables 1 and 2, the magnetic characteristics were 1.58 T in saturation magnetic flux density  $B_s$  and 26 in magnetic permeability  $\mu$ , strength of the base material was 18 kgf/mm<sup>2</sup>, volume resistivity was  $8.3 \times 10^{-3}$   $\Omega$ cm, and formability of metal plating layer was X. SEM-EDS analysis confirmed that the grains were bonded with one another via the metal oxide (oxide layer) formed on the surfaces of the grains by the heat treatment, and the oxide layer was an oxide containing an element that oxidizes more easily than iron (here chromium) by a quantity larger than that in the alloy grains.

#### Example 7

Inductors were obtained in the same manner as in Example 1, except that the treatment temperature in the standard atmosphere was changed to 1000° C. The obtained results of measurement and judgment are shown in Table 1. As shown in Tables 1 and 2, the magnetic characteristics were 1.50 T in saturation magnetic flux density  $B_s$  and 50 in magnetic permeability  $\mu$ , strength of the base material was 20 kgf/mm<sup>2</sup>, volume resistivity was  $2.0 \times 10^2$   $\Omega$ cm, and formability of metal plating layer was X. In this reference example where the heat treatment temperature was raised, the 3-point bending rupture stress was higher, but the volume resistivity was lower, compared to Example 1. SEM-EDS analysis confirmed that the grains were bonded with one another via the metal oxide (oxide layer) formed on the surfaces of the grains by the heat treatment, and the oxide layer was an oxide containing an element that oxidizes more easily than iron (here chromium) by a quantity larger than that in the alloy grains.

#### Example 8

Evaluation samples were created in the same manner as in Example 1, except that the composition ratio of material grains was changed to 9.5 percent by weight of silicon, 5.5 percent by weight of aluminum and 85 percent by weight of iron. The obtained results of measurement and judgment are shown in Tables 1 and 2. As shown in Tables 1 and 2, the magnetic characteristics were 0.77 T in saturation magnetic flux density  $B_s$  and 32 in magnetic permeability  $\mu$ , strength of

20

the base material was 1.4 kgf/mm<sup>2</sup>, volume resistivity was  $8.0 \times 10^3$   $\Omega$ cm, and formability of metal plating layer was X. The volume resistivity was low and no metal plating layer could be formed on the baked conductive layer constituting the external conductive film. Also, SEM-EDS analysis confirmed that the grains were bonded with one another via the metal oxide (oxide layer) formed on the surfaces of the grains by the heat treatment, and the oxide layer was an oxide containing an element that oxidizes more easily than iron (here aluminum) by a quantity larger than that in the alloy grains.

#### Comparative Example 1

Evaluation samples were created in the same manner as in Example 1, except that the composition ratio of material grains was changed to 1 percent by weight of chromium, 6.5 percent by weight of silicon and 92.5 percent by weight of iron. The obtained results of measurement and judgment are shown in Tables 1 and 2. As shown in Tables 1 and 2, the magnetic characteristics were 1.36 T in saturation magnetic flux density  $B_s$  and 17 in magnetic permeability  $\mu$ , strength of the base material was 4.2 kgf/mm<sup>2</sup>, volume resistivity was  $4.9 \times 10^1$   $\Omega$ cm, and formability of metal plating layer was X. In this comparative example where the Cr content was less than 2 percent by weight based on the result of SEM-EDS analysis, the metal oxide layer generated on the surfaces of grains by the heat treatment was not an oxide containing an element that oxidizes more easily than iron (here chromium) by a quantity larger than that in the alloy grains, which resulted in the low volume resistivity.

#### Reference Example 1

Evaluation samples were created in the same manner as in Example 1, except that heat treatment was not performed. The obtained results of measurement and judgment are shown in Tables 1 and 2. As shown in Tables 1 and 2, the magnetic characteristics were 1.50 T in saturation magnetic flux density  $B_s$  and 35 in magnetic permeability  $\mu$ , strength of the base material was 0.54 kgf/mm<sup>2</sup>, and volume resistivity was  $1.4 \times 10^5$   $\Omega$ cm. Note that in this reference example, no sample was created or evaluated with regards to formability of a metal plating layer. The result of SEM-EDS analysis found that no metal oxide layer was generated on the surface of grains in this reference example. This explains why the volume resistivity was slightly lower than that in the examples.

#### Reference Example 2

Evaluation samples were created in the same manner as in Example 1, except that the temperature of heat treatment in the standard atmosphere was changed to 300° C. The obtained results of measurement and judgment are shown in Tables 1 and 2. As shown in Tables 1 and 2, the magnetic characteristics were 1.50 T in saturation magnetic flux density  $B_s$  and 35 in magnetic permeability  $\mu$ , strength of the base material was 0.83 kgf/mm<sup>2</sup>, and volume resistivity was  $1.4 \times 10^5$   $\Omega$ cm. Note that in this reference example, no sample was created or evaluated with regards to formability of a metal plating layer. In this reference example, SEM-EDS analysis confirmed that an oxide layer constituted by metal oxide was not sufficiently formed on the surfaces of the grains, because the heat treatment temperature was lower than 400° C. This explains why the volume resistivity was slightly lower than that in the examples.

Next, an example of laminated type is given. Using the same alloy grains in Example 1, a coil-type electronic component was created which had 20 layers, a shape of 3.2 mm×1.6 mm×0.8 mm in size, and a coil inside the base material. First, a mixture containing 85 percent by weight of alloy metal grains, 13 percent by weight of butyl carbitol (solvent) and 2 percent by weight of polyvinyl butylal (binder) was processed into a sheet shape of 40  $\mu\text{m}$  in thickness using a die-coater, after which conductive paste containing 85 percent by weight of Ag grains, 13 percent by weight of butyl carbitol (solvent) and 2 percent by weight of polyvinyl butylal (binder) was applied on the sheet to form conductive patterns. Next, sheets on which conductive patterns were formed, each produced as above, were stacked on top of each other and pressed under a pressure of 2 tons/cm<sup>2</sup> to obtain a laminate. The laminate was heat-treated at 800° C. for 2 hours in the standard atmosphere to obtain a base material. Paste containing Ag was then applied on the based material in which a coil had been formed inside, specifically on the surfaces where the coil's pullout parts were exposed and also

on the installation surfaces, after which the base material was heat-treated at 700° C. for 10 minutes to obtain a coil-type electronic component with a metal plating layer that had been formed. The magnetic characteristics were 1.41 T in saturation magnetic flux density  $B_s$  and 15 in magnetic permeability  $\mu$ . The magnetic permeability  $\mu$  was 13 before the heat treatment. Ni was used to form the metal plating layer. SEM-EDS analysis confirmed that the grains were bonded with one another via the metal oxide (oxide layer) formed on the surfaces of the grains by the heat treatment, and the oxide layer was an oxide containing an element that oxidizes more easily than iron (here chromium) by a quantity larger than that in the alloy grains. Additionally, it was confirmed that in Examples 1 to 4, there were grains wherein the thickness of an oxide layer bonding the grains with one another was thicker than that of an oxide layer on the surfaces of the alloy grains. It was confirmed that in Examples 5 and 6, there were grains wherein the thickness of an oxide layer bonding the grains with one another was thinner than that of an oxide layer on the surfaces of the alloy grains. It was confirmed that in Examples 1 to 8, there were grains wherein the thickness of an oxide layer was 50 nanometers or greater.

TABLE 1

| Composition [wt %] | Grain size d50 |     |     |      | Heat treatment temperature |        | 3-point bending rupture stress |       | Volume resistivity     | Formability of metal  |               |
|--------------------|----------------|-----|-----|------|----------------------------|--------|--------------------------------|-------|------------------------|-----------------------|---------------|
|                    | Cr             | Si  | Al  | Fe   | [um]                       | [° C.] | [T]                            | $\mu$ | [kgf/mm <sup>2</sup> ] | [ $\Omega\text{cm}$ ] | plating layer |
| Example 1          | 5              | 3   | —   | 92   | 10                         | 700    | 1.51                           | 45    | 7.4                    | $4.2 \times 10^5$     | ○             |
| Example 2          | 3              | 5   | —   | 92   | 10                         | 700    | 1.46                           | 43    | 2.8                    | $2.0 \times 10^5$     | ○             |
| Example 3          | 5              | 3   | —   | 92   | 6                          | 700    | 1.45                           | 27    | 6.6                    | $3.0 \times 10^5$     | ○             |
| Example 4          | 5              | 3   | —   | 92   | 3                          | 700    | 1.38                           | 20    | 7.6                    | $7.0 \times 10^5$     | ○             |
| Example 5          | 9.5            | 3   | —   | 87.5 | 10                         | 700    | 1.36                           | 33    | 7.4                    | $4.7 \times 10^{-3}$  | ×             |
| Example 6          | 5              | 1   | —   | 94   | 10                         | 700    | 1.58                           | 26    | 18                     | $8.3 \times 10^{-3}$  | ×             |
| Example 7          | 5              | 3   | —   | 92   | 10                         | 1000   | 1.50                           | 50    | 20                     | $2.0 \times 10^2$     | ×             |
| Example 8          | —              | 9.5 | 5.5 | 85   | 10                         | 700    | 0.77                           | 32    | 1.4                    | $8.0 \times 10^3$     | ×             |
| Comp. Ex. 1        | 1              | 6.5 | —   | 92.5 | 10                         | 700    | 1.36                           | 17    | 4.2                    | $4.9 \times 10^1$     | ×             |
| Ref. Ex. 1         | 5              | 3   | —   | 92   | 10                         | —      | 1.50                           | 35    | 0.54                   | $1.4 \times 10^5$     | —             |
| Ref. Ex. 2         | 5              | 3   | —   | 92   | 10                         | 300    | 1.50                           | 35    | 0.83                   | $1.4 \times 10^5$     | —             |

TABLE 2

| Heat treatment temperature [° C.] | Heat Treatment Temperatures and 3-point Bending Rupture Stresses [kgf/mm <sup>2</sup> ] |           |           |           |           |           |           |           | Comp. Example 1 |
|-----------------------------------|-----------------------------------------------------------------------------------------|-----------|-----------|-----------|-----------|-----------|-----------|-----------|-----------------|
|                                   | Example 1                                                                               | Example 2 | Example 3 | Example 4 | Example 5 | Example 6 | Example 8 | Example 1 |                 |
| 25                                | 0.54                                                                                    | 0.48      | 0.51      | 0.52      | 0.48      | 0.53      | 0.25      | 0.55      |                 |
| 150                               | 1.1                                                                                     | 1.2       | 1.1       | 1.3       | 1.0       | 1.3       | 0.89      | 1.2       |                 |
| 200                               | 0.45                                                                                    | 0.31      | 0.42      | 0.55      | 0.48      | 0.72      | 0.19      | 0.58      |                 |
| 300                               | 0.83                                                                                    | 0.72      | 0.90      | 1.01      | 0.92      | 0.92      | 0.23      | 0.82      |                 |
| 500                               | 3.4                                                                                     | 1.2       | 2.0       | 3.7       | 3.6       | 5.7       | 0.26      | 2.4       |                 |
| 600                               | 4.5                                                                                     | 1.7       | 3.5       | 5.1       | 4.9       | 8.0       | 0.43      | 3.9       |                 |
| 700                               | 7.4                                                                                     | 2.8       | 6.6       | 7.6       | 7.4       | 18        | 1.4       | 4.2       |                 |
| 800                               | 12                                                                                      | 4.5       | 10        | 16        | 17        | 24        | 5.7       | 6.5       |                 |
| 1000                              | 20                                                                                      | 7.3       | 15        | 27        | 28        | 33        | 7.8       | 8.2       |                 |

\* The heat treatment temperature of 1000° C. in Example 1 corresponds to the heat treatment temperature used in Example 7.

TABLE 3

| Heat treatment temperature [° C.] | Heat Treatment Temperatures and $\mu$ |           |           |           |           |           |           |           | Comp. Example 1 |
|-----------------------------------|---------------------------------------|-----------|-----------|-----------|-----------|-----------|-----------|-----------|-----------------|
|                                   | Example 1                             | Example 2 | Example 3 | Example 4 | Example 5 | Example 6 | Example 8 | Example 1 |                 |
| 25                                | 35                                    | 32        | 23        | 19        | 28        | 23        | 24        | 30        |                 |
| 700                               | 45                                    | 43.0      | 27        | 20        | 33        | 26        | 32        | 17        |                 |
| $\Delta\mu$                       | 29                                    | 36        | 17        | 7         | 18        | 13        | 33        | -43       |                 |

$\Delta\mu = (\mu \text{ at heat treatment temperature } 700^\circ \text{ C.} - \mu \text{ at heat treatment temperature } 25^\circ \text{ C.})/\mu \text{ at heat treatment temperature } 25^\circ \text{ C.} \times 100$

A base material using a soft magnetic alloy for an electronic component conforming to the present invention, as well as an electronic component made of such base material, are ideally suited to compact electronic components that can be installed on the surface of a circuit board. In particular, they are ideally suited to the size reduction of power inductors through which high current flows.

## DESCRIPTION OF THE SYMBOLS

- 1: Grain 2: Oxide layer 3: Void 10, 10': Base materials using a soft magnetic alloy for an electronic component 11: Drum-type core 11a: Winding center 11b: Flange part 12: Sheet-shaped core 14: External conductive film 14a: Baked conductive film layer 14b: Ni plating layer 14c: Sn plating layer 15: Coil 15a: Winding part 15b: End (joined part) 20: Electronic component (winding-type chip inductor) 31: Laminated chip 34: External conductive film 35: Internal coil 40: Electronic component (laminated chip inductor) d1: Long-axis dimension d2: Short-axis dimension

What is claimed is:

1. A coil-type electronic component having a base material and a coil inside or on the surface of the base material, wherein the base material is constituted by a group of grains of a soft magnetic alloy containing iron, silicon and other element that oxidizes more easily than iron; the surface of each soft magnetic alloy grain has an oxide layer formed on the surface of each soft magnetic alloy grain as a result of oxidization of the grain; said oxide layer contains the other element that oxidizes more easily than iron in a quantity larger than that in the soft magnetic alloy grain; and grains are bonded with one another via said oxide layer,

wherein the aforementioned oxide layer includes in this order a first oxide layer where the content of the aforementioned iron component decreases while the content of the aforementioned element that oxidizes easily increases, and a second oxide layer where the content of the aforementioned iron component decreases and the content of the aforementioned element that oxidizes easily also decreases, as viewed outwardly from the aforementioned alloy grain.

2. A coil-type electronic component according to claim 1, wherein the oxide layer via which the soft magnetic alloy grains are bonded with one another is thicker than an oxide layer other than the bonding oxide layer on the surface of the soft magnetic alloy grains.

3. A coil-type electronic component according to claim 1, wherein the oxide layer via which the soft magnetic alloy grains are bonded with one another is thinner than an oxide layer other than the bonding oxide layer on the surface of the soft magnetic alloy grains.

4. A coil-type electronic component according to claim 1, wherein the oxide layer formed on at least some of the soft magnetic grains has a thickness of at least 50 nanometers.

5. A coil-type electronic component according to claim 1, wherein the aforementioned oxide layer bonding the aforementioned grains is constituted by the same phase.

6. A coil-type electronic component according to claim 1, wherein the aforementioned element that oxidizes more easily than iron is chromium.

7. A coil-type electronic component according to claim 1, wherein the aforementioned element that oxidizes more easily than iron is aluminum.

8. A coil-type electronic component according to claim 6, wherein the aforementioned soft magnetic alloy has a composition of 2 to 8 percent by weight of chromium, 1.5 to 7 percent by weight of silicon, and 88 to 96.5 percent by weight of iron.

9. A coil-type electronic component according to claim 7, wherein the aforementioned soft magnetic alloy has a composition of 2 to 8 percent by weight of aluminum, 1.5 to 12 percent by weight of silicon, and 80 to 96.5 percent by weight of iron.

10. A coil-type electronic component according to claim 1, wherein the average size of the soft magnetic grain based on arithmetic mean is 30 micrometers or less.

11. A coil-type electronic component according to claim 1, wherein the aforementioned first oxide layer, as viewed outwardly from the aforementioned alloy grain, has an inflection point with respect to the content of the aforementioned silicon.

12. A coil-type electronic component according to claim 1, wherein the peak strength ratio of the element that oxidizes more easily than iron, relative to iron, in the oxide layer is higher than the peak strength ratio of the element that oxidizes more easily than iron, relative to iron, in the aforementioned grain, based on calculation by the ZAF method through energy diffusion X-ray analysis using a scanning electron microscope.

13. A coil-type electronic component according to claim 1, wherein the aforementioned coil has its end electrically connected to a conductive film formed on the surface of the aforementioned base material.

14. A coil-type electronic component having a base material and a coil, wherein the base material is constituted by a group of grains of a soft magnetic alloy; the surface of each soft magnetic alloy grain has an oxide layer formed on the surface of each soft magnetic alloy grain as a result of oxidization of the grain; said oxide layer contains a quantity of a metal that oxidizes more easily than iron, said quantity being larger than that in the alloy grains; the grains are bonded with one another via said oxide layer; and a coil said coil is formed inside the base material,

wherein the aforementioned oxide layer includes in this order a first oxide layer where the content of the aforementioned iron component decreases while the content of the aforementioned element that oxidizes easily increases, and a second oxide layer where the content of the aforementioned iron component decreases and the content of the aforementioned element that oxidizes easily also decreases, as viewed outwardly from the aforementioned alloy grain.

15. A coil-type electronic component according to claim 14, wherein the coil conductor forms conductive patterns and is sintered simultaneously with the base material.

16. A coil-type electronic component according to claim 14, wherein the metal that oxidizes more easily than iron in the oxide layer is chromium.

17. A coil-type electronic component according to claim 14, wherein the metal that oxidizes more easily than iron in the oxide layer is aluminum.